

E. L. DUFOURCQ.

PROCESS FOR TREATMENT OF PRECIOUS METAL ORES FOR EXTRACTING THEIR VALUES.

APPLICATION FILED NOV. 7, 1911.

1,133,110.

Patented Mar. 23, 1915.

Fig. 1.



Fig. 2.



Fig. 3.



Witnesses.

J. P. Collard  
J. George Barry

Inventor:

Edward L. Dufourcq,  
by his attorney  
Franklin Ward

# UNITED STATES PATENT OFFICE.

EDWARD L. DUFURCQ, OF NEW YORK, N. Y.

## PROCESS FOR TREATMENT OF PRECIOUS-METAL ORES FOR EXTRACTING THEIR VALUES.

1,133,110.

Specification of Letters Patent. Patented Mar. 23, 1915.

Application filed November 7, 1911. Serial No. 659,018.

To all whom it may concern:

Be it known that I, EDWARD L. DUFURCQ, a citizen of the United States, and resident of the borough of Manhattan, in the city and State of New York, have invented a new and useful Improvement in Processes for Treatment of Precious-Metal Ores for Extracting Their Values, of which the following is a specification.

10 The object of my invention is to produce a new process for the treatment of precious metal ores for extracting their values, which process consists in dissolving the precious metals of an ore of these metals, such, for instance, as gold or silver ore, by means of a solution of cyanid of sodium or potassium or other solvent, continuously by means of agitation by compressed air introduced into the solvent; such particles of the ore under 15 treatment as may be shown in the course of the process to be of too large a size to be treated effectively, being removed from the action of the solvent solution and the oxidizing effect of the compressed air, for subsequent re-treatment, thus permitting the remaining particles of the ore to be more quickly dissolved with a very considerably reduced consumption of the cyanid salt or other solvent agent.

20 Three different forms of apparatus which may be effectively used for carrying out the process are represented in the accompanying drawings, in which—

Figure 1 represents in diagram three successive V-boxes having their downtime and uptake sides inclined, Fig. 2 shows in diagram four successive V-boxes having their downtime sides vertical and their uptake sides inclined, and Fig. 3 shows in diagram 40 four V-boxes with their downtime sides inclined and their uptake sides vertical.

The downtime sides of the boxes are denoted by 1 and their uptake sides by 2. A vertically arranged baffle board 3 is located 45 in each V-box, the bottom of which baffle board is adjusted the desired distance from the bottom of the V-box.

The bottom of each V-box is provided with a device for permitting the removal of the coarser particles, which device is herein shown as an outlet pipe 4 having a valve 5 therein to open and close the same. Each V-box is also provided with means for introducing jets or streams of compressed air upwardly along the uptake side of the V-box.

This is provided for in the illustration shown herein by a series of pipes 6, one only of which is shown in each V-box, said pipes being provided with a valve 7 for controlling the passage of compressed air therethrough.

In carrying out the process, the ore is subjected to continuous successive treatments in the solvent solution in a plurality of successive V-boxes, the number of said V-boxes being varied to suit different requirements. The mass is passed downwardly along the downtime side of the V-box by gravity and then upwardly along the uptake side of the V-box by means of the upwardly directed jets of compressed air, the overflow from the first V-box passing into the downtime side of the second V-box of the series and from thence through as many boxes as may be desired. The coarser particles which are found to be too large for proper treatment will remain in the bottoms of these V-boxes where they may be removed through the outlet pipes 4. These coarser particles may be prepared for subsequent re-treatment by grinding them to a finer consistency or, if their values are unprofitable, they may be discarded. If so desired, the process may be carried out without the removal of the coarser particles if this be found unnecessary in the treatment of certain particular ores, the treatment of the ores in successive boxes by successive jets of air serving in itself to secure a more complete and rapid extraction of the values.

What I claim is:—

1. The herein described process for treatment of precious metal ores for extracting their values consisting in passing the ore and solution continuously through successive baths, agitating the mass in each bath by means of an air blast, and removing the coarser particles from the mass in any one or more of the said baths.

2. The herein described process for treatment of precious metal ores for extracting their values, consisting, first, in treating the ore with a solvent, second, passing the resulting mass into the first of a series of open-faced V boxes, third, agitating the mass and forcing it from one V box to another by means of a series of air blasts located in the V boxes, and fourth, removing the coarser particles from the mass in any one of said boxes as the process goes on.

3. The herein described process for treatment of precious metal ores for extracting their values, consisting, first, in treating the ore with a suitable solvent, second, passing 5 the parts of the dissolved ore and its solvent solution downwardly along the downtime side of an open-faced V box around a baffle-board, third, in applying a blast of compressed air to the mass when it reaches the 10 bottom of the V box to agitate it and force it upwardly along the uptake side of the V box into a second V box and continuing the

same treatment through a series of V boxes, and fourth, removing the coarser particles from the mass from time to time as it passes 15 through said series of boxes.

In testimony that I claim the foregoing as my invention, I have signed my name in presence of two witnesses, this third day of November 1911.

EDWARD L. DUFOURCQ.

Witnesses:

F. GEORGE BARRY,  
C. S. SUNDGREN.